

Feb. 9, 1937.

J. L. SCHUELER ET AL

2,070,554

PROCESS OF TREATING GALVANIZED COATINGS

Filed May 6, 1935



Inventors:

Julian L. Schueler,  
and Chatmer L. Heninger,  
By Banning & Banning  
Attys.

## UNITED STATES PATENT OFFICE

2,070,554

## PROCESS OF TREATING GALVANIZED COATINGS

Julian L. Schueler and Chalmer L. Heninger,  
Kokomo, Ind., assignors to Continental Steel  
Corporation, Kokomo, Ind., a corporation of  
Indiana

Application May 6, 1935, Serial No. 19,930

3 Claims. (Cl. 91—70.2)

This invention relates to a treatment for a galvanized coating to be performed by preference when the coating is freshly applied while it is still in a molten state. Specifically we raise the 5 temperature of such a coating, or at least maintain the coating in a fully liquid condition, and then impart thereto a sudden and brief chilling treatment in a manner which will produce beneficial results. This has been performed successfully 10 in connection with continuous galvanizing operations on wires, wire fabrics, wire fencing, etc., but may possibly with equal advantage be applied to sheets or articles which are galvanized by a semi-continuous or intermittent process.

15 In the ensuing description we shall explain our invention in relation to the treatment of wires by way of example. It is well known that a sudden chilling of a coating freshly applied to a wire will produce an attractive appearance.

20 There is usually the penalty, however, of an increased liability for the coating to dust and to crack and peel from the wire, particularly when it is bent or fabricated. It is difficult, if not impossible, to chill such a coating for the purpose 25 of obtaining a bright appearance without incurring some of the disadvantages just referred to.

According to our process the wire upon emerging 30 from a bath of molten spelter may be moved through a high temperature zone to maintain the coating in a fully liquid condition or even to further liquefy the coating. The wire is then passed immediately through a thin chilling curtain of water, steam, air or other gaseous medium. The speed of wire travel in relation to 35 the temperature of this chilling curtain and the thickness thereof is such as to prevent any substantial chilling of the wire itself which forms the base for the coating. This step of coating 40 conditioning may be carried out with a flame apparatus, as suggested in the Schueler Reissue Patent No. 19,209, wherein the coating is subjected to a constant impingement with the possibility of a progressively decreasing tempera- 45 ture; or it may be carried out with a heat treater, as suggested in the Herman Patent No. 1,430,648, wherein there is no impingement and the temperature of the surrounding inert air is substantially uniform. These two treatments, while es- 50 sentially different, are alike in the one respect that they serve to raise the temperature of the coating and increase its liquidity to a point somewhat above that which may obtain in the bath, and hence are available in the practice of our 55 invention.

After this preliminary treatment which we regard as desirable although perhaps not necessary in all cases, the coating on the wire is subjected to a sudden and brief chilling. Experience with wires so treated indicates that there is little or no dusting of the coating in consequence. The surface of the coating is rendered harder and better suited for various purposes. 5

As indicative of certain apparatus which is suitable for carrying out this invention, we have 10 shown in Figure 1 a longitudinal section through one end of a galvanizing bath adjacent which is a flame apparatus having at its exit end a means for producing a thin water curtain;

Fig. 2 is a similar view in which a heat treater 15 is substituted for the flame apparatus; and

Fig. 3 is an enlarged longitudinal view in section through the water curtain apparatus.

A number of wires *w*, arranged side by side, may be passed through a galvanized bath *B* near 20 the exit end of which is a coating regulator *R* which removes dross, skimmings and coating in excess of that which is desired. Passing from the coating regulator the wire enters immediately into a flame apparatus *F* where the temperature of the coating may be raised. If desired, the flame may be so controlled that the temperatures in this unit of the apparatus will progressively decrease toward the exit end. Immediately upon emerging from the flame apparatus 25 the wire passes through a chilling medium *C* which we prefer should be in the form of a thin curtain of water. Substantially the same apparatus is shown in Fig. 2 where a heat treater *H* is substituted for the flame apparatus. 30

The chilling apparatus shown in Fig. 3 comprises a pipe *p* having connection with a water source. Surrounding this pipe is a jacket *j* the ends of which are connected to a fitting *f* with an associated gland *g* and packing nut *n*. The 40 space within the jacket is accordingly sealed at every point.

Extending through the pipe, preferably on its under side, are openings *4* through which water may enter the jacketed space. If desired, baffles 45 *5* may be arranged in the pipe to check the flow of water therethrough. The jacket is provided on its upper side with one or more orifices the form and arrangement of which may be varied as found desirable. One such opening *6* may be provided adjacent each wire *w* as indicated at the left end of Fig. 3; we may also employ two openings *7* having their axes converging toward the proximate wire; and it may be feasible to use a narrow slit *8* extending in proximity to the adjacent wire, 50 55

or an elongated slit 9 extending for a distance equal to the spacing between two or more wires, as indicated at the right end of Fig. 3. Any one or more of those forms and arrangements of orifices 5 may be employed. The jacketed pipe is arranged above a trough T having one or more drain openings d.

In operation a thin curtain of water is projected upwardly from the orifice in the jacket to 10 a point above the wires thereover. The water curtain proceeds both up and down, so as to contact with the wires at every circumferential point. The chilling effect, therefore, is sudden, brief and uniform. The speed of wire travel, perhaps 15 50 to 125 feet per minute, is such that the effect of chilling is confined to the coating alone. It does not penetrate through to the steel base upon which the coating is carried, or, at most, its effect will reach only the exterior surface of 20 the base.

At the moment that the coating is subjected to this brief chilling action, the temperature of the coating is considerably above its melting point. In fact, it may be several hundred degrees (Fahrenheit) 25 thereabove. Whether or not this is responsible for the beneficial results we cannot say, but it is certain that the coating thus treated is free from the detrimental effects of enhanced flaking, chilling and dusting so common with 30 coatings which are chilled by ordinary processes. We would have it understood, however, that the important point is not necessarily the raising of the coating temperature, but a maintained liquefaction thereof up to the moment that chilling 35 takes place; and that the chilling itself, whether produced by water, air, steam or other medium, is relatively sudden, brief and uniformly applied so as to affect the coating alone, or at most only the exterior surface of the base whereon the coating is carried.

We claim:

1. In the art of continuously galvanizing wire by the hot dipping process, the steps of advancing the wire with the applied zinc coating still molten through a zone of relatively high 5 temperature sufficient to raise the temperature of the molten coating to a point beyond that previously acquired, and thereafter immediately advancing the coating through a thin water curtain the temperature and volume of which in relation 10 to the speed of wire travel is so regulated as to chill the coating but not the wire base interiorly thereof.

2. In the art of continuously galvanizing wire by the hot dipping process, the steps of subjecting successive portions of a molten coating freshly applied to a wire while the wire is in longitudinal motion, to treatment by a regulator whereby to partially decoat the wire, in then subjecting successive portions of the coating of reduced amount 15 while still molten to the action of heat sufficient to raise further the temperature of the coating, and immediately thereafter in subjecting successive portions of the molten coating so raised in temperature to a sudden chilling action whose 20 intensity and duration is such as not to affect appreciably the temperature of the wire base to 25 which the coating is applied.

3. In the art of galvanizing, the steps of subjecting an article upon which a zinc coating is 30 still molten to the action of heat sufficient to raise further the temperature of the coating, and immediately thereafter in subjecting the coating to a chilling action whose intensity and duration 35 is insufficient to impart an appreciable chill to the article whereon the coating is carried.

JULIAN L. SCHUELER.  
CHALMER L. HENINGER.